

1

3,449,119

## HIGH VANADIUM ALLOYS

Frederick C. Holtz, Jr., Evanston, Ill., assignor, by mesne assignments, to the United States of America as represented by the Secretary of the Navy  
 No Drawing. Filed Nov. 15, 1966, Ser. No. 594,627  
 Int. Cl. C22c 1/02, 27/00; C21d 1/78  
 U.S. Cl. 75—134

9 Claims

### ABSTRACT OF THE DISCLOSURE

A vanadium-columbium-titanium alloy with small percentages of silicon and carbon characterized by high tensile strength between —320° F. and 2000° F.

This invention relates to a vanadium base alloy containing columbium and titanium with small additives of silicon and carbon.

Previous vanadium alloy studies had indicated that vanadium-columbium base compositions had attractive short-time strength properties in the 1800° to 2400° F. range. Limited testing at temperatures as low as —452° F. (—259° C.) showed these materials to be unusually strong and ductile. The present work was aimed at producing dispersion-strengthened compositions which would not only have good cryogenic properties but also good retention of strength at temperatures above that at which the nickel and cobalt base superalloys are used. Because of their comparatively low melting point, these alloys were not expected to be as strong as columbium, molybdenum, tantalum or other refractory alloys at temperatures in excess of 2400° F. However, the excellent fabrication characteristics and the ability to form reliable silicide oxidation-protective coatings indicate high potential for use over a wide range of temperatures. The development of space craft finds a need for alloys which will retain their strength at both low and high temperatures.

The object of the present invention is to provide an alloy or group of alloys which excell in fabricability, ductility and high strength over a range from —320° F. to at least 2000° F.

Another object of the present invention is to provide a group of alloys which will have high strength at extremes of low and high temperatures and which will form oxidation-protective coating.

Still another object of the present invention is to provide a vanadium based alloy containing columbium and titanium and additives of silicon and carbon.

Other objects will be apparent from the subsequent disclosures and appended claims.

The alloys which are the subject of this invention are based on a V-Cb-Ti system with small additives of Si and C.

#### Materials used:

In the experimental procedures a single lot of vanadium melting stock was used with the following analysis of the V.

2

|          |       |
|----------|-------|
| Oxygen   | 0.040 |
| Nitrogen | 0.028 |
| Carbon   | 0.040 |
| Hydrogen | 0.004 |
| Iron     | 0.050 |
| Silicon  | 0.020 |

Non-consumable electrode arc-melted ingots of this melting stock had hardness levels in the VPN (10 kg.) 160—170 range.

10 Columbium sheet used as melting stock was electron-beam melted and had less than 0.01 wt. percent total oxygen and nitrogen. Titanium sheet of similar purity was used. Minor additions such as zirconium, silicon were made from high-purity commercial melting stock. Carbon was added as an arc-melted 95V-5C master alloy.

Percentages of materials used:

|           | Percent               |
|-----------|-----------------------|
| Columbium | 15-20                 |
| Titanium  | 5-10                  |
| Silicon   | 0.25-0.75             |
| Carbon    | 0.75-0.25             |
| Vanadium  | Remainder to make 100 |

### INGOT PREPARATION

#### (1) Melting

20 All of the compositions were prepared by nonconsumable-electrode arc-melting under a highly purified argon atmosphere. Ingot weights ranged from 150 to 200 grams, depending on density, and the ingots were inverted and remelted five times to insure good homogeneity. These ingots were approximately 0.4 in. thick by 2.4 in. in diameter.

#### (2) Thermal homogenization

25 The arc-melted ingots were thermally homogenized in a tantalum-element resistance-heated furnace. These heat treatments were conducted under vacuum ( $10^{-5}$  torr or better) or in argon which was purified by passing the gas through hot titanium sponge and a liquid nitrogen trap. After heating for the desired length of time, the ingots were lowered from the hot zone and cooled by a stream of flowing argon at a rate of approximately 400° F./min.

#### (3) Ingot fabrication

30 The initial ingot breakdown for nearly all of the alloys was achieved by hammer forging. The ingots were jacketed in 0.030 in. thick stainless steel, then evacuated. Hammer forging was done at 2350°-2400° F. on a mechanical drop hammer. Reductions in thickness of 30 to 40% were used to obtain a final forged thickness of 0.25 to 0.30 inch. The more difficult-to-work alloys required reheating to achieve this reduction. After forging, the jackets were stripped and any edge or surface cracks were removed by grinding. The conditioned ingots were then cold-rolled, in most cases with intermediate vacuum annealing, to sheet ranging in thickness from 0.004 to 0.027 in. Rolling reductions were initially 10% per pass, although smaller reductions were used when the sheet was less than 0.030 in. thick. A list of representative compositions together with the processing methods and results of ingot fabrication is presented in Table I.

TABLE I.—VANADIUM ALLOY FABRICATION DATA

| Composition, wt. percent       | Density, lb./in. <sup>3</sup> | Fabrication Procedure <sup>a</sup>                | Results                                                             |
|--------------------------------|-------------------------------|---------------------------------------------------|---------------------------------------------------------------------|
| V-15 Cb-10 Ti-0.5 Si-0.15 C    | 0.22                          | HF-CR-Ann-Cr                                      | Good sheet, 0.009 in.                                               |
| V-20 Cb-Ti-0.25 Si-0.1 C       | 0.23                          | {TH 2,800° F.-HF<br>HF-CR                         | Cracked.<br>Good sheet, 0.027 in.                                   |
| V-20 Cb-5 Ti-0.5 Si-0.1 C      | 0.23                          | {TH 2,800° F.-HF<br>HF-CR                         | Cracked.<br>Good sheet, 0.027 in.                                   |
| V-20 Cb-7.5 Ti-0.5 Si-0.15 C   | 0.22                          | HF-CR-Ann-CR                                      | Good sheet, 0.009 in.                                               |
| V-20 Cb-10 Ti-0.375 Si-0.075 C | 0.22                          | HF-CR-Ann-CR                                      | Good sheet, 0.025 in.                                               |
| V-20 Cb-10 Ti-0.5 Si-0.05 C    | 0.22                          | HF-CR-Ann-CR                                      | Good sheet, 0.008 in.                                               |
| V-20 Cb-10 Ti-0.5 Si-0.075 C   | 0.22                          | HF-CR-Ann-CR                                      | Good sheet, 0.010 in.                                               |
| V-20 Cb-10 Ti-0.5 Si-0.15 C    | 0.22                          | HF-CR-Ann-CR                                      | Good sheet, 0.009 in.                                               |
| V-20 Cb-10 Ti-0.4 Si-0.2 C     | 0.22                          | HF-CR                                             | Severe edge cracks at 0.04 in.                                      |
| V-20 Cb-10 Ti-0.5 Si-0.2 C     | 0.22                          | HF-CR-Ann-CR                                      | Good sheet, 0.009 in.                                               |
| V-20 Cb-10 Ti-0.7 Si-0.15 C    | 0.22                          | HF-CR-Ann-CR                                      | Do.<br>Cracked.                                                     |
| V-20 Cb-10 Ti-0.75 Si-0.15 C   | 0.22                          | {TH 2,800° F.-HF<br>HF-CR-Ann-CR                  | Good sheet, 0.018 in.                                               |
| V-20 Cb-10 Ti-0.4 Si-0.25 C    | 0.22                          | {TH 2,600° F.-HF CR<br>{TH 2,300° F.-HF-CR-Ann-CR | Extensive cracking at 0.2 in.<br>Moderate edge cracking at 0.03 in. |
| V-60 Cb-1 Ti                   | 0.27                          | CR-Ann-CR                                         | Good sheet, 0.027 in.                                               |

<sup>a</sup> TH=Thermal homogenization, 3 hr. at 2,800° F., 4 hr. at 2,300 and 2,600° F.; HF=hammer forge; Ann=Vacuum anneal, 1/2 hr. at 2,000 to 2,400° F.; CR=Cold roll.

### RECRYSTALLIZATION

Alloys based on V-Cb-Ti were evaluated for recrystallization behavior. Sheet specimens were cold-rolled to reductions in thickness of about 80%, then annealed in

at temperatures from 1200 to 1600° F. Most of the aged specimens were evaluated by room temperature tensile tests. Table III presents data for three alloys containing varying amounts of silicon and carbon.

TABLE III.—AGING RESPONSE OF HIGH-VANADIUM ALLOYS <sup>a</sup>

| Treatment        | V-20 Cb-10 Ti-0.5 Si-0.15 C |                 | V-20 Cb-10 Ti-0.7 Si-0.15 C |                 | V-20 Cb-10 Ti-0.5 Si-0.2 C |                 |
|------------------|-----------------------------|-----------------|-----------------------------|-----------------|----------------------------|-----------------|
|                  | UTS, p.s.i.                 | Elong., percent | UTS, p.s.i.                 | Elong., percent | UTS, p.s.i.                | Elong., percent |
| As cold rolled   | 181,000                     | 1.5             | 187,000                     | (b)             | 186,000                    | 1.0             |
| 1,200° F.-4 hr.  | 197,000                     | 2.5             | 203,000                     | 3.0             | 197,000                    | 3.0             |
| 1,200° F.-8 hr.  | 199,000                     | 3.0             | 214,000                     | 2.5             | 193,000                    | 2.0             |
| 1,200° F.-16 hr. | 194,000                     | 3.0             | 202,000                     | (b)             | 202,000                    | 4.5             |
| 1,200° F.-48 hr. | 208,000                     | 3.0             | 213,000                     | 5.0             | 201,000                    | (b)             |
| 1,200° F.-96 hr. | 185,000                     | 4.5             | 190,000                     | 7.0             | 180,000                    | 5.0             |
| 1,300° F.-1 hr   | 187,000                     | 7.0             | 200,000                     | 6.5             | 192,000                    | 5.0             |
| 1,300° F.-4 hr   | 180,000                     | 8.0             | 189,000                     | 6.0             | 183,000                    | 7.0             |
| 2,000° F.-1/2 hr | 123,000                     | 24.0            | 117,000                     | 17.0            | 121,000                    | 20.5            |

<sup>a</sup> Cold rolled to 0.008 in. prior to indicated treatment.

<sup>b</sup> Broke outside of gage marks.

a vacuum for 30 minutes at temperatures in the 1600–2400° F. range. The extent of crystallization was determined by metallographic observation, and hardness measurements were also taken on the annealed specimens. Table II lists the lowest temperatures at which complete crystallization occurred after 30 minutes annealing treatments conducted at 100° F. intervals. Hardness data for the fully crystallized specimens are also included.

TABLE II.—RECRYSTALLIZATION AND HARDNESS DATA FOR VANADIUM ALLOYS

| Composition, wt. percent     | Recrystallization Temp., ° F. | Hardness, VPN |
|------------------------------|-------------------------------|---------------|
| V-15 Cb-10 Ti-0.5 Si-0.15 C  | 1,700                         | 280           |
| V-20 Cb-7.5 Ti-0.5 Si-0.15 C | 1,700                         | 280           |
| V-20 Cb-10 Ti-0.5 Si-0.15 C  | 1,700                         | 280           |
| V-20 Cb-10 Ti-0.4 Si-0.2 C   | 1,800                         | 269           |
| V-20 Cb-10 Ti-0.5 Si-0.2 C   | 1,800                         | 289           |
| V-20 Cb-10 Ti-0.7 Si-0.15 C  | 1,700                         | 293           |

### AGING RESPONSE

Studies of aging behavior were carried out on selected alloys of the V-Cb-Ti system. Sheet specimens were fully annealed for 30 minutes at 2000° F. The specimens were cooled from the annealing temperature at a rate of about 250° F./min. to room temperature, then cold-rolled to reductions in thickness of 60–80%. Aging was conducted

40 Solution-annealed specimens of two V-Cb-Ti base alloys were also aged and evaluated for room-temperature tensile properties. Solutionizing was done for 40 min. at 2000° F. followed by water quenching. Aging at 1100° and 1200° F. produced the following results for the alloy V-Cb-10Ti-0.5Si-0.075C.

| Treatment                                       | Ultimate Tensile Strength, p.s.i. | Elongation, percent |
|-------------------------------------------------|-----------------------------------|---------------------|
|                                                 |                                   |                     |
| 2,000° F.-40 min., W.Q.                         | 124,000                           | 19                  |
| 2,000° F.-40 min., W.Q.; aged 1,100° F., 24 hr. | 148,000                           | 13                  |
| 2,400° F.-40 min., W.Q.; aged 1,200° F., 4 hr.  | 135,000                           | 15                  |

50 Similar results were obtained for the V-20Cb-10Ti-0.5Si-0.05C alloy. These data indicate that solution annealing followed by aging does not produce strength levels as high as those obtained by cold-rolling followed by aging, although the tensile elongations are higher.

### CRYOGENIC TENSILE PROPERTIES

The alloys were tested for tensile strength at temperatures as low as that of liquid nitrogen (−320° F.). The tested specimens had a 1/4 by 1 in. gage section, and were 60 tested at a strain rate of 0.005 in./in./min. The results are shown in Table IV.

TABLE IV.—TENSILE DATA FOR VANADIUM ALLOYS AT LIQUID NITROGEN TEMPERATURE (−320° F.)

| Composition, wt. percent    | Treatment <sup>a</sup> | Ultimate Tensile Strength, p.s.i. | Total Elongation, percent | Density Corrected Strength, UTS/(lb./in. <sup>2</sup> ) |
|-----------------------------|------------------------|-----------------------------------|---------------------------|---------------------------------------------------------|
| V-20 Cb-10 Ti-0.5 Si-0.15 C | Annealed               | 205,000                           | 26.2                      | 919,000                                                 |
|                             | Aged 1,200° F., 24 hr. | 270,000                           | 14.2                      | 1,210,000                                               |
|                             | Aged 1,300° F., 1 hr.  | 275,000                           | 12.0                      | 1,233,000                                               |
| V-20 Cb-10 Ti-0.5 Si-0.2 C  | Annealed <sup>b</sup>  | 205,000                           | 23.8                      | 928,000                                                 |
|                             | Aged 1,200° F., 24 hr. | 280,000                           | 11.8                      | 1,267,000                                               |
|                             | Aged 1,300° F., 1 hr.  | 275,000                           | 12.8                      | 1,245,000                                               |
| V-20 Cb-10 Ti-0.7 Si-0.15 C | Annealed <sup>b</sup>  | 210,000                           | 25.8                      | 942,000                                                 |
|                             | Aged 1,200° F., 14 hr. | 275,000                           | 11.7                      | 1,233,000                                               |
|                             | Aged 1,300° F., 1 hr.  | 290,000                           | 12.0                      | 1,300,000                                               |
| V-20 Cb-10 Ti-0.4 Si-0.25 C | Aged 1,200° F., 48 hr. | 253,000                           | 11.2                      | 1,145,000                                               |
|                             | Aged 1,300° F., 2 hr.  | 239,000                           | 14.8                      | 1,080,000                                               |

<sup>a</sup> Aging treatments after 60–80% reduction by cold rolling.

<sup>b</sup> Fully recrystallized—2000° F., 30 min.

TABLE V.—ROOM-TEMPERATURE TENSILE DATA FOR FULLY ANNEALED VANADIUM ALLOYS.

| Composition, wt. percent            | Ultimate Tensile Strength, p.s.i. | 0.2% Offset Yield Strength, p.s.i. | Elongation, percent | Density-Corrected Strength, UTS/(lb./in. <sup>2</sup> ) |
|-------------------------------------|-----------------------------------|------------------------------------|---------------------|---------------------------------------------------------|
| V-15 Cb-10 Ti-0.5 Si-0.15 C-----    | 111,000                           | 92,500                             | 22                  | 506,000                                                 |
| V-20 Cb-5 Ti-0.25 Si-0.1 C b-----   | 108,000                           | 92,000                             | 25                  | 476,000                                                 |
| V-20 Cb-5 Ti-0.5 Si-0.1 C-----      | 116,000                           | 99,500                             | 27                  | 511,000                                                 |
| V-20 Cb-7.5 Ti-0.5 Si-0.15 C-----   | 114,000                           | 96,000                             | 21.5                | 509,000                                                 |
| V-20 Cb-10 Ti-0.375 Si-0.075 C----- | 114,000                           | 102,000                            | 24                  | 512,000                                                 |
| V-20 Cb-10 Ti-0.5 Si-0.05 C-----    | 114,500                           | 102,500                            | 20                  | 520,000                                                 |
| V-20 Cb-10 Ti-0.5 Si-0.075 C-----   | 116,000                           | 102,500                            | 18                  | 528,000                                                 |
| V-20 Cb-10 Ti-0.5 Si-0.15 C-----    | 123,000                           | 113,000                            | 24                  | 552,000                                                 |
| V-20 Cb-10 Ti-0.5 Si-0.2 C-----     | 121,000                           | 102,500                            | 20.5                | 548,000                                                 |
| V-20 Cb-10 Ti-0.7 Si-0.15 C-----    | 117,000                           | 102,000                            | 17                  | 525,000                                                 |
| V-20 Cb-10 Ti-0.75 Si-0.15 C b----- | 132,000                           | 120,000                            | 17                  | 594,000                                                 |

<sup>a</sup> Vacuum annealed 2,000° F., 30 min., unless otherwise noted.  
<sup>b</sup> 2,200° F.—10 min.

## ROOM TEMPERATURE TENSILE PROPERTIES

Tests conducted at room temperature are shown in Table V. The results in Table V were obtained on 0.008 to 0.025 in. thick sheet which was cooled from the annealing temperature to below visible heat at a rate of approximately 250° F./min. Both carbon and silicon strengthened the V-20Cb-10Ti base to a moderate degree. The strongest alloy, V-20Cb-10Ti-0.75Si-0.15C, had a density corrected strength of 594,000 in. This high strength was due to the high silicon content and possibly to the fact that the 10-min, anneal at 2200° F. produced retention of more strengthening elements in solid solution than was obtained at 2000° F. annealing temperature used for most of the alloys. The effects of various annealing treatments on the composition V-20Cb-10Ti-0.5Si-0.075C are shown below:

| Treatment                                    | Ultimate<br>Tensile<br>Strength,<br>p.s.i. | Elonga-<br>tion,<br>percent |
|----------------------------------------------|--------------------------------------------|-----------------------------|
| 1,800° F., 10 min., cool at 250° F./min..... | 117,000                                    | 21                          |
| 2,000° F., 30 min., cool at 250° F./min..... | 116,000                                    | 18                          |
| 2,000° F., 40 min., water quench.....        | 124,000                                    | 19                          |

## ELEVATED-TEMPERATURE TENSILE PROPERTIES

Tests for tensile strength were conducted on sheet specimens of alloys at 1200, 1800, 2000, 2200 and 2400° F. using a strain rate of 0.05 in./in./min. The sheet stock was approximately 0.008 in. thick and the specimens were tested in the as-rolled, fully annealed and cold-rolled and aged condition. The results of tensile tests for tantalum-free high-vanadium alloys are presented in Table VI.

TABLE VI.—ELEVATED-TEMPERATURE TENSILE DATA FOR HIGH-VANADIUM V-Cb-Ti BASE ALLOYS

| Composition, wt. percent     | Treatment                                | Test Temp., °F. | Ultimate Tensile Strength, p.s.i. | Elongation, percent | Density-Corrected Strength, UTS/(lb./in. <sup>2</sup> ) |
|------------------------------|------------------------------------------|-----------------|-----------------------------------|---------------------|---------------------------------------------------------|
| V-20 Cb-10 Ti-0.5 Si-0.05 C  | Annealed 2,000° F., 30 min. <sup>a</sup> | 1,800           | 30,000                            | 69                  | 136,000                                                 |
|                              | Annealed 2,000° F., 30 min., WQ          | 1,800           | 59,000                            | 26                  | 266,000                                                 |
| V-20 Cb-10 Ti-0.5 Si-0.075 C | Annealed 2,000° F., 30 min. <sup>a</sup> | 2,000           | 27,000                            | 86                  | 123,000                                                 |
|                              | Annealed 2,000° F., 30 min., WQ          | 1,800           | 57,000                            | 24                  | 250,000                                                 |
| V-20 Cb-10 Ti-0.5 Si-0.15 C  | Cold rolled 80%                          | 2,000           | 27,000                            | 79                  | 123,000                                                 |
|                              | do                                       | 1,200           | 185,000                           | <1                  | 830,000                                                 |
|                              | Annealed 2,000° F., 30 min. <sup>a</sup> | 1,800           | 31,800                            | 100                 | 142,000                                                 |
| V-20 Cb-10 Ti-1.4 Si-0.2 C   | do <sup>a</sup>                          | 1,800           | 52,300                            | 34                  | 234,000                                                 |
|                              | Cold rolled 80%                          | 2,000           | 40,000                            | 70                  | 179,000                                                 |
|                              | Annealed 2,000° F., 30 min. <sup>a</sup> | 1,800           | 33,200                            | 26                  | 150,000                                                 |
| V-20 Cb-10 Ti-0.5 Si-0.2 C   | do <sup>a</sup>                          | 1,800           | 59,000                            | 34                  | 267,000                                                 |
|                              | Cold rolled; aged 1,200° F., 48 hrs.     | 1,200           | 182,000                           | 1                   | 852,000                                                 |
| V-20 Cb-10 Ti-0.7 Si-0.15 C  | Annealed 2,000° F., 30 min. <sup>a</sup> | 1,800           | 61,800                            | 28                  | 280,000                                                 |
|                              | Cold rolled                              | 1,800           | 25,500                            | 125                 | 114,000                                                 |

<sup>a</sup> Cooled at 250° F./min.

### References Cited

UNITED STATES PATENTS

- |           |        |               |       |        |
|-----------|--------|---------------|-------|--------|
| 2,886,431 | 5/1959 | Smith et al.  | ----- | 75-134 |
| 3,038,798 | 6/1962 | Berger et al. | ----- | 75-174 |
| 3,136,631 | 6/1964 | Wlodek        | ----- | 74-134 |

RICHARD O. DEAN, *Primary Examiner.*

UNITED STATES PATENT OFFICE  
CERTIFICATE OF CORRECTION

Patent No. 3,449,119 Dated June 10, 1969  
Inventor(s) FREDERICK C. HOLTZ, JR.

It is certified that error appears in the above-identified patent  
and that said Letters Patent are hereby corrected as shown below:

✓

Claim 7, line 2, after "7.5Ti-" insert  
-- 0.5Si- --.

SIGNED AND  
SEALED

DEC 30 1969

(SEAL)

Attest:

Edward M. Fletcher, Jr.

Attesting Officer

WILLIAM E. SCHUYLER, JR.  
Commissioner of Patents